

## UNITED STATES PATENT OFFICE

2,631,929

STABILIZING VANADIUM CONTAINING  
FUEL OILS

Thomas Charles Gordon Thorpe, Hampton Hill,  
and Edwin Mathieson Dodds, Wantage, Eng-  
land, assignors to Standard Oil Development  
Company, a corporation of Delaware

No Drawing. Application December 6, 1949, Se-  
rial No. 131,506. In Great Britain October 21,  
1948

2 Claims. (Cl. 44—79.)

1

The present invention relates to improved hydrocarbon fuel oils of the type which contain vanadium compounds, which compounds are liable to be deposited as solid vanadium pentoxide on combustion.

Heavy residual fuel oils have, for a long time, been used in steam-raising boilers and the like. Combustion systems of this type are comparatively crude and the deposition of ash from the fuel inside the system, while reducing its overall efficiency, is not a problem of major importance. More recently residual fuels have been proposed for use in more sensitively adjusted systems such as gas turbines and diesel engines, and in systems such as these where the tolerance between moving parts is small and where restriction to gas flow must be avoided, the build-up of deposits is a serious problem.

Residual fuel oils from certain crudes, especially Venezuelan, contain substantial amounts of vanadium. While some of the ash-forming constituents are present as solid impurities and may be largely removed by such methods as filtration or centrifuging, it appears that the vanadium is present in oil-soluble form, probably as vanadium naphthenates, and accordingly cannot be removed by simple mechanical methods.

When such fuels are burnt in boiler furnaces through atomizing burners of conventional type, it is found that deposits containing a very large proportion of vanadium pentoxide are formed in the system. These deposits are undesirable since they reduce the thermal efficiency and probably help to catalyze the reaction  $2\text{SO}_2 + \text{O}_2 \rightarrow 2\text{SO}_3$ , which is generally considered to be the cause of flue gas corrosion. Nevertheless, the deposits may be cleaned off periodically without undue difficulty, and their presence does not prevent the furnace from working.

In contrast to this, when vanadium-containing oils are burnt in gas turbines or diesel engines, the deposits tend to build up on the turbine blades or round the exhaust valves respectively, and in due course this may reduce the efficiency of the engine to an extent which necessitates dismantling and cleaning it. Furthermore, with high vanadium fuels this necessity may arise with uneconomic frequency.

In summary, therefore, the presence of vanadium compounds in residual fuels is always disadvantageous and the disadvantages become more pronounced as the degree of precision of the equipment in which they are used increases.

The object of the present invention is to provide an improved fuel in which this disadvantage

2

is alleviated or obviated altogether, and the use of which will tend to remove existing vanadium oxide deposits when used in equipment in which they have already been formed, and according thereto there is incorporated in the vanadium-containing fuel oil a minor proportion of an oil-soluble organic halogen compound. Also included within the scope of the invention is the method of operating combustion apparatus in which

10 vanadium-containing fuel oil is burnt which comprises carrying out the combustion in the presence of a minor proportion of an oil-soluble organic halogen compound. In this method of operating there may be used the improved fuel already described, or the vanadium-containing fuel may be used unblended, and the organic halogen compound, e. g., in the form of a relatively concentrated solution in mineral oil, injected into the fuel system either before or into the combustion chamber, the main thing being to ensure that the halogen compound is present during the actual combustion of the fuel. As a modification of the process, volatile inorganic compounds such as  $\text{HCl}$  could be employed in this manner.

20 25 The halides and oxyhalides of vanadium are reasonably volatile at the combustion temperatures involved (900–1200° F.) and it appears that they are probably formed in preference to vanadium oxide, provided that the halogen is present during the combustion. While it is not intended to be bound by the accuracy or otherwise of any theory put forward, it is considered that injection of the halogen compound at a later stage of the combustion cycle, or in other words 30 35 into the hot exhaust gases would be considerably less efficient. Nevertheless, particularly in the case of furnaces, there may be no clear cut line of demarcation between combustion and flue gases, and it is within the scope of the present 40 45 invention to inject the halogen compound into the gas stream at any point where the temperature is sufficiently high to cause substantial scavenging of the vanadium. As already indicated, however, it is preferred to have the halogen present in the fuel before combustion.

The amount of halogen compound to be added will depend upon the amount of vanadium present and in general should be in excess of the amount theoretically required. At the same time, 50 the question of corrosion of the turbine or furnace should be considered, so that excessive amounts of halogen should not be used. For any normal fuel it will be found that an amount of additive equivalent to  $\frac{1}{2}\%$  chlorine by weight will provide a substantial theoretical excess, and that

quantities of the order of 0.1% or even less will still provide ample halogen for effective scavenging. Owing to the low cost of fuel oil, it is desirable that the amount of additive be kept as low as practicable, and for the same reason it is preferred to use relatively available highly halogenated compounds such as carbon tetrachloride, ethylene dichloride, chloroform and hexachloroethane. Other compounds such as chlorobenzenes may be used but the aliphatic compounds appear to be more effective. While the use of halogens other than chlorine is theoretically practicable, they are undesirable on economic grounds, and their physical properties are less well suited to the purpose of the invention than are those of the chlorides and oxychlorides.

Preliminary laboratory tests indicated that the reaction of organic halogen compounds, of the type mentioned above, with vanadium pentoxide started below red heat and became more vigorous as the temperature was increased to red heat. In order to confirm that this result was representative of what would occur in practice, a pair of experimental runs were made on an open-cycle gas turbine. In such a turbine, the combustion gases pass through the turbine system, in contrast to a closed cycle turbine in which the operating medium is hot air. When run on gas oil, the unit can be run more or less indefinitely with satisfactory results.

For test, there was selected a fuel having a high ash content with the ash preponderantly vanadium. The fuel, a heavy fuel oil, had the following characteristics:

|                             |               |
|-----------------------------|---------------|
| Specific gravity            | 0.9634        |
| Redwood viscosity at 100° F | secs 966      |
| Ash                         | per cent 0.06 |
| Sulphur                     | do 2.2        |
| Ash analysis:               |               |

|                                           |                |
|-------------------------------------------|----------------|
| Vanadium as V <sub>2</sub> O <sub>5</sub> | per cent 81.8  |
| Iron as Fe <sub>2</sub> O <sub>3</sub>    | do 5.6         |
| Nickel, calcium and sodium                | not determined |

In the first run, this fuel was used without any additive and starting with a clean turbine. The test terminated after 30 hours' running, with a steady power drop, which, when the test finished had reached 45% (i. e., the final power output was 55% of the initial power output).

On opening up the turbine for inspection, it was found to be very heavily fouled indeed both on the stators and on the rotors, with the severity of fouling decreasing steadily from a maximum at the high temperature end to a minimum at about the fourth stage, after which no more than a greenish colouration was visible. The blades showed no signs of corrosion. The deposits were heaviest on the concave side of the first row of rotors and stators and on the convex side of subsequent rows. Samples of these deposits were removed and analysed and proved to have the following composition:

|                                           | Deposit on 1st and 2nd row blades | Deposit on 3rd and 4th row blades |
|-------------------------------------------|-----------------------------------|-----------------------------------|
| Vanadium as V <sub>2</sub> O <sub>5</sub> | 72.7%                             | 60.1%                             |
| Iron as Fe <sub>2</sub> O <sub>3</sub>    | 7.9%                              | 5.5%                              |
| Nickel as NiO                             | 6.8%                              | 4.3%                              |
| Calcium as CaO                            | 4.5%                              | 14.3%                             |
| Sodium as Na <sub>2</sub> O               | 1.1%                              | 3.3%                              |
| Sulphate as SO <sub>4</sub>               | 2.8%                              | 8.3%                              |
| Moisture                                  | Present                           | Present                           |

From this result it will be quite apparent that the presence of the vanadium in the fuel oil has

rendered the turbine virtually inoperative in as short a period as 30 hours.

The turbine was then cleaned and the test run was repeated using the same fuel but with the addition of 1/2% by weight of carbon tetrachloride. This additive has the merits of high chlorine content and ready availability, but its boiling point is rather low if the fuel is to undergo prolonged storage.

Using this modified fuel, the turbine ran perfectly normally for 70 hours with no measurable power drop. Since it was considered that any potential adverse effects would have begun to show themselves after 70 hours' running, and since there was no trace of any such effect, the test was stopped deliberately after the 70 hours and the turbine opened for inspection.

In comparison with the first test the amount of deposit was extremely small and confined to the first row of stator and of rotor blades. Furthermore, what deposits there were on the blades were flaky and loose. No corrosion due to halogen was observed. For comparison with the previous deposits, analysis of the deposit from the first row of stator blades is given below:

|                                           |               |
|-------------------------------------------|---------------|
| Vanadium as V <sub>2</sub> O <sub>5</sub> | per cent 77.1 |
| Iron as Fe <sub>2</sub> O <sub>3</sub>    | do 3.6        |
| Nickel as NiO                             | do 5.1        |
| Calcium as CaO                            | do 1.7        |
| Sodium as Na <sub>2</sub> O               | do 2.1        |
| Sulphate as SO <sub>4</sub>               | do 8.4        |
| Chloride as Cl                            | do 1.1        |
| Moisture                                  | Present       |

Owing to the construction of the turbine and the nature of the deposits it was not feasible to conduct the test on quantitative lines and relate the quantity of vanadium deposited on the engine in each run to that contained in the fuel burnt during the run. Nevertheless it was obvious to the eye that the amount of deposits in the second run was a very small fraction of that of the first run, despite the fact that over twice as much fuel was burnt. In addition, there is the incontrovertible fact that in the first run, the engine was forced to a virtual standstill after only 30 hours' running, whereas the second run could apparently have continued indefinitely.

It will be clear from this test that the improved fuel of the present invention does most effectively suppress vanadium deposition, and that equally beneficial results would be experienced when using it in steam boilers or diesel engines. When used for diesel engines, in particular marine diesels, it is desirable that the fuel should also be centrifuged (e. g., treated in a centrifugal purifier and/or clarifier) to remove oil-insoluble matter. Furthermore, when used for gas turbines or furnaces it may be desirable to inject liquid water into the system periodically in order to remove deposits, primarily consisting of sodium salts, which may have built up.

What is claimed is:

1. A fuel composition consisting of a vanadium-containing heavy fuel oil and 0.5% by weight of an oil-soluble halogen compound chosen from the class consisting of carbon tetrachloride, ethylene dichloride, chloroform and hexachloroethane.
2. Composition according to claim 1 in which the halogen compound is carbon tetrachloride.

THOMAS CHARLES GORDON THORPE.  
EDWIN MATHIESON DODDS.

(References on following page)

5

## REFERENCES CITED

The following references are of record in the  
file of this patent:

## UNITED STATES PATENTS

5

| Number    | Name    | Date          | Number    |
|-----------|---------|---------------|-----------|
| 238,867   | Draper  | Mar. 15, 1881 | 2,218,281 |
| 1,098,412 | Shaw    | June 2, 1914  | 2,441,751 |
| 1,637,007 | North   | July 26, 1927 | 2,460,700 |
| 2,078,958 | Lysholm | May 4, 1937   | 10        |

6

| Name      | Date          |
|-----------|---------------|
| De Ridder | Oct. 15, 1940 |
| Broggi    | May 18, 1948  |
| Lyons     | Feb. 1, 1949  |

## FOREIGN PATENTS

| Country       | Date          |
|---------------|---------------|
| Great Britain | Apr. 14, 1936 |
| Great Britain | Dec. 5, 1938  |